

# United States Patent Office

2,725,292

Patented Nov. 29, 1955

1

2,725,292

## COLORED COUPLERS CONTAINING SOLUBILIZING GROUPS

Bruce Graham, Los Altos, Calif., and Paul W. Vittum and Arnold Weissberger, Rochester, N. Y., assignors to Eastman Kodak Company, Rochester, N. Y., a corporation of New Jersey

No Drawing. Application May 15, 1952,  
Serial No. 288,022

6 Claims. (Cl. 95—6)

This invention relates to color photography and particularly to colored couplers for use in photographic processes.

Color-forming compounds which react with the development product of aromatic amino developing agents to form colored images upon photographic development are well known. Generally, these color-forming compounds of couplers are colorless or substantially colorless. This lack of color is usually desirable where the coupler is to be incorporated in the emulsion layer and the unused coupler remains after formation of the colored image. When the coupler is used in the developing solution, it may be colored without detriment to the final image and certain colored couplers have been used in this way.

Couplers which are in themselves more or less strongly colored, and which contain a chromophore group which is split off or destroyed during and by means of the coupling reaction, with the result that the original color of the coupler is destroyed and a new dye is formed upon coupling, are disclosed in Glass, Vittum and Weissberger U. S. Patents 2,453,661; 2,455,169; 2,455,170 and 2,521,908.

If the colored couplers are to be used in aqueous colloidal emulsion carriers, the couplers must also contain groups conferring water solubility such as sulfonic acid or carboxylic acid groups. These lyophilic groups may be present in the coupler portion of the molecule or the phenylazo portion of the molecule or both. Compounds containing lyophilic groups have been described in our prior application Serial No. 260,098, filed December 5, 1951, now Patent No. 2,657,134.

We have now found that a different type of solubilizing group may be used in colored couplers to accomplish useful results in color photography. The new colored couplers which are the subject of the present invention contain an azo portion in which the solubilizing group is separated from the arylazo unit by a connecting chain of such constitution that it can release electrons toward the arylazo unit and thus facilitate the coupling function. These compounds may be represented by the following general formula:

Coupler—N=N—A—B—C

2

in which A is an aryl group, B is an electron releasing substituent on A, and C is a solubilizing, lyophilic group.

More specifically, our invention involves the use of coupler compounds having the formula



in which R represents the atoms necessary to complete a pyrazolone, phenol or naphthol ring, C represents the carbon atom in the 4-position of each of said rings, X represents an oxygen atom or a single chemical bond, and Z represents a carboxylic acid or sulfonic acid group or a water-soluble salt or alkyl ester of these groups.

The water-soluble salt is usually an alkali metal salt such as sodium or potassium. The alkyl ester is usually a methyl or ethyl ester.

The following examples illustrate couplers which may be used according to our invention:



35 1-phenyl-3-(3-[2-(2,4-di-tert-amylphenoxy)-5-(2-sulfobenzamido)benzamido]-4-[4-(carboxymethoxy)phenylazo]-5-pyrazolone



45 1-phenyl-3-(3-[2-(2,4-di-tert-amylphenoxy)-5-(2-sulfobenzamido)benzamido]-4-[4-(carboxymethyl)phenylazo]-5-pyrazolone

50 1-hydroxy-4-[4-(carboxymethoxy)phenylazo]-N-(4-[2-(2,4-di-



(4)



1-hydroxy-4-[4-(carboxymethyl)phenylazo]-5-(3-sulfobenzamido)benzamido-2-naphthamide

(5)



1-[4-(4-tert-butylphenoxy)phenyl]-3-[α-(4-tert-butylphenoxy)propionamido]-4-[4-carboxymethyl]phenylazo-5-pyrazolone

(6)



1-hydroxy-3'-carbethoxy-4-[4-(carboxymethyl)phenylazo]-4'-(2,4-di-tert-amylphenoxy)-2-naphthanilide

(7)



1-[4-(4-tert-butylphenoxy)phenyl]-3-[α-(4-tert-butylphenoxy)propionamido]-4-[sulfomethyl]phenylazo-5-pyrazolone

(8)



1-phenyl-3-[2-(2,4-di-tert-amylphenoxy)-5-(2-sulfobenzamido)benzamido]-4-[4-(sulfomethyl)phenylazo]-5-pyrazolone

The couplers of our invention are miscible with aqueous colloid emulsion carriers such as gelatin or polyvinyl alcohol and can therefore be incorporated directly into the usual photographic emulsions. When incorporated directly in this way the couplers are used in the form of their water soluble salt. They may also be used in the ester form in processes such as those of Mannes and Godowsky U. S. Patent 2,304,940 and Jelley and Vittum



U. S. Patent 2,322,027. When used in this way they are incorporated in a solvent which is then dispersed in the

emulsion and it is generally desirable that all of the acid groups be esterified. However, in certain cases, a free acid group may be present in the molecule when the 30 couplers are incorporated in this way, if there are sufficient solvent-solubilizing groups in the molecule as in the case of compound No. 5.

In order to facilitate crystallization of the couplers it is often convenient to prepare the carboxylic acids in 35 the form of their esters and the sulfonic acids in the form of their sulfonyl chlorides. If the compounds are to be incorporated directly in the gelatin, these groups can then be hydrolyzed just before the couplers are added to the emulsion.

40 The preparation of our compounds will now be described.

The parent colorless couplers (without the arylazo group) are known compounds or are prepared as follows:

Compounds 1, 2 and 8 are described in U. S. application Serial No. 260,098, now U. S. Patent 2,657,134, Example 4.

Compounds 3 and 4 are described in U. S. application Serial No. 260,098, now U. S. Patent 2,657,134, Example 1.

Compounds 5 and 7 are described in U. S. Patent 2,369,489, Example 47.

60 Parent compound No. 6 was prepared as follows: 2-(2,4-di-tert-amylphenoxy)-5-nitrobenzoyl chloride was converted to the ethyl ester, M. P. 40-45° C., by refluxing it in ethyl alcohol. This was reduced to the amino derivative by use of 10% palladium on carbon in petroleum ether at room temperature. The amino compound was condensed with 1-hydroxy-2-naphthoate at 150-200° C. to yield 1-hydroxy-[3'-carbethoxy-4'-(2,4-di-tert-amylphenoxy)-1-2-naphthanilide, M. P. 152-153°.

70 The anilines used in the preparation of the diazo derivatives for reaction with the parent couplers are easily obtained. p-Aminophenylacetic acid is commercially available. Other anilines were prepared as follows:

*p-Sulfomethylaniline.*—p-Nitrobenzylsulfonic acid was made by the action of p-nitrobenzyl chloride on sodium bisulfite in the presence of sodium hydroxide. The reduction was accomplished by dissolving the p-nitrobenzyl-

sulfonic acid in cold concentrated ammonium hydroxide and passing in hydrogen sulfide. The salt of the desired aniline was obtained by concentration of the reaction mixture.

*p*-Aminophenoxyacetic acid.—*p*-Nitrophenoxyacetic acid [J. Am. Chem Soc., 39, 2424 (1917)] was reduced in aqueous solution over 5% palladium on carbon. The free amine was converted to the hydrochloride for storage. M. P. 222-223° C. The esters of these acids can be easily prepared by the conventional methods.

The final colored couplers were prepared in general by dissolving the appropriate colorless coupler in pyridine at 0° C. and treating the resulting solution with the diazotized aniline derivative at 0° C. The resulting dye was isolated by drowning the reaction mixture in cold, dilute hydrochloric acid. The products were washed in cold water on a filter. The following specific method for the preparation of compound No. 1 is typical:

*Example 1*

A solution of 83 parts of colorless coupler No. 1 in 300 parts of pyridine was cooled to 0° C. and treated with a cold solution of *p*-carboxymethoxybenzenediazonium chloride prepared as follows: *p*-aminophenoxyacetic acid hydrochloride (21 parts) in 250 parts of water and 13 parts of concentrated hydrochloric acid was cooled to 0° C. and treated with a solution of 7.3 parts of sodium nitrite in 30 parts of water. The aqueous pyridine dye solution was allowed to stand overnight. It was then poured into a mixture of 500 parts of concentrated hydrochloric acid in 1000 parts of ice. The product was collected and washed repeatedly with cold water on the filter. It was then triturated with water, and collected and washed again. Yield 88 parts of orange dye which sinters above 150° C. and melts to a spongy mass at about 170° C.

The physical properties of the amorphous colored couplers are listed below:

M. P.

|            |                               |
|------------|-------------------------------|
| Compound 1 | Amorphous softens 150-170° C. |
| Compound 2 | Softens 160-190°.             |
| Compound 3 | Sinters>180°, M. 205-210°.    |
| Compound 4 | Sinters>190°, M. ca. 205°.    |
| Compound 5 | Sinters>140.                  |
| Compound 6 | 250-255°.                     |
| Compound 7 | M. 273° (from acetic acid).   |
| Compound 8 | Sinters>200°, M. 250-260°.    |

Our couplers are intended to be incorporated in one of the emulsion layers of a multilayer coating in order to secure the masking effects described in Hanson U. S. Patent 2,449,966. The Hanson process involves a color correction method in which a colored coupler is incorporated in the photographic emulsion layer prior to exposure and upon development is converted to a colored image where the layer is exposed. The coupler remaining in the unexposed portions of the layer retains its original color and by suitable choice of the color of the original coupler and the color of the final dye image, a masking or correction effect can be obtained.

The following example illustrates the incorporation of one of our couplers directly in a gelatino-silver halide emulsion:

*Example 2*

A 5-gram sample of the coupler having the structure of compound 3 was wet with 15 ml. of ethyl alcohol and heated with 5 ml. of 20% sodium hydroxide solution. The addition of 200 ml. of water produced a clear solution which remained clear when the pH was reduced to 6.5-7.0. The neutralized solution was mixed with about 250 ml. of a silver halide emulsion and coated according to standard practice. An exposure on this material after normal negative processing gave a negative cyan image and an orange-yellow positive image.

The following example illustrates the incorporation of 75 where R is a mononuclear aryl radical.

one of our couplers in a solvent dispersion in a gelatino-silver halide emulsion.

*Example 3*

5 A solution of seven grams of the compound 5 was prepared by heating with 25 ml. of dibutylphthalate at 165° C. A dispersion of this solution was prepared by milling with 90 ml. of 10% aqueous gelatin solution and 20 ml. of 5% Alkanol B at 45° C. This dispersion was 10 mixed with 125 ml. of water and approximately 250 ml. of a silver halide emulsion and then coated according to standard practice. Exposed coatings of this material when processed in the usual negative color development process gave a negative magenta image and a positive yellow image.

Various photographic developing agents can be employed with the couplers of our invention. The primary aromatic amino developing agents are generally suitable including the phenylene-diamines and aminophenols.

20 The alkyl phenylenediamines may be substituted in the amino group as well as in the ring. Suitable compounds are diethyl paraphenylenediamine, monomethyl para-phenylenediamine, dimethyl paraphenylenediamine and para-aminophenol. These compounds are usually employed in the salt form, such as the hydrochloride or the sulphate which are more stable than the free amines. All of these compounds have a primary amino group which enables the oxidation product of the developer to couple with the color-forming compounds to form dye 25 images.

30 The following developing solution is suitable for developing gelatino-silver halide layers containing colored couplers according to our invention incorporated either directly in the emulsion or in solvent dispersion:

|                                     | Grams |
|-------------------------------------|-------|
| 2-amino-5-diethyl-amino toluene HCl | 2     |
| Sodium sulphite                     | 2     |
| Sodium carbonate                    | 20    |
| Potassium bromide                   | 2     |
| Water to 1 liter.                   |       |

Where we refer in the claims to "pyrazolone, phenol and naphthol rings," it is to be understood that we intend to include substituted as well as unsubstituted rings, as well known in the art and as illustrated by the specific 45 examples above.

It will be understood that the examples and modifications set forth herein are illustrative only and that our invention is to be taken as limited only by the scope of the appended claims.

50 We claim:

1. A silver halide emulsion containing a coupler compound having the formula:



where R represents the atoms necessary to complete a ring selected from the class consisting of pyrazolone, phenol and naphthol, C represents the carbon atom in the 4-position of said ring, X is selected from the class consisting of —O— and a single chemical bond para to the azo group, and Z is selected from the class consisting of —COOH and —SO3H and their water-soluble salts and alkyl esters.

60 2. A silver halide emulsion containing a coupler compound having the formula:



The following example illustrates the incorporation of 75 where R is a mononuclear aryl radical.

3. A silver halide emulsion containing a coupler compound having the formula:



where R is an aralkyl radical.

4. A silver halide emulsion containing a coupler compound having the formula:



where R is an aryloxyalkyl radical and R' is a mononuclear aryl radical.

5. A silver halide emulsion containing a coupler compound having the formula:



where R and R' are mononuclear aryl radicals.

6. A silver halide emulsion containing a coupler compound having the formula



where R is an aryloxyalkyl radical and R' is a mononuclear aryl radical.

10 References Cited in the file of this patent

## UNITED STATES PATENTS

2,455,169 Glass \_\_\_\_\_ Nov. 30, 1948

## FOREIGN PATENTS

598,174 Great Britain \_\_\_\_\_ Feb. 12, 1948

598,657 Great Britain \_\_\_\_\_ Feb. 24, 1948

627,814 Great Britain \_\_\_\_\_ Aug. 16, 1949

267,707 Switzerland \_\_\_\_\_ Apr. 1, 1950